# EUROPEAN PATENT SPECIFICATION

(11) **EP 3 194 641 B1**
(45) Date of publication and mention of the grant of the patent: **22.12.2021**
(21) Application number: 15842267.5
(22) Date of filing: 18.09.2015
(51) Int. Cl.: C25D 1/00, C25D 3/56, C25D 5/14, C25D 5/18, C25D 5/00

(54) **NICKEL-CHROMIUM NANOLAMINATE COATING OR CLADDING HAVING HIGH HARDNESS**
NICKEL-CHROM-NANOLAMINATBESCHICHTUNG ODER -KASCIERUNG MIT HOHER HÄRTE
REVÊTEMENT NANOSTRATIFIÉ OU GAINAGE DE NICKEL-CHROME PRÉSENTANT UNE DURETÉE ÉLEVÉE

(30) Priority: 18.09.2014 US 201462052437 P
(43) Date of publication of application: 26.07.2017
(73) Proprietor: Modumetal, Inc., Seattle, Washington 98103 (US)
(72) Inventor: SKLAR, Glenn, Seattle, Washington 98144 (US)
(74) Representative: Herr, Ulrike Maria
(86) International application number: PCT/US2015/050910
(87) International publication number: WO 2016/044708

(56) References cited:
- WO-A1-2014/145588
- US-A- 4 461 680
- US-A- 4 975 337
- US-B2- 8 152 985
- HUANG ET AL: "Characterization of Cr-Ni multilayers electroplated from a chromium(III)-nickel(II) bath using pulse current", SCRIPTA MATERIALIA, ELSEVIER, AMSTERDAM, NL, vol. 57, no. 1, 24 April 2007 (2007-04-24) , pages 61-64, XP022044412, ISSN: 1359-6462, DOI: 10.1016/J.SCRIPTAMAT.2007.02.004
- HUANG C A ET AL: "Hardness variation and annealing behavior of a Cr-Ni multilayer electroplated in a trivalent chromium-based bath", SURFACE AND COATINGS TECHNOLOGY, ELSEVIER BV, AMSTERDAM, NL, vol. 203, no. 20-21, 15 July 2009 (2009-07-15), pages 3320-3324, XP026142653, ISSN: 0257-8972, DOI: 10.1016/J.SURFCOAT.2009.04.011 [retrieved on 2009-04-18]
- ETMINANFAR M R ET AL: "Corrosion resistance of multilayer coatings of nanolayered Cr/Ni electrodeposited from Cr(III) Ni(II) bath", THIN SOLID FILMS, ELSEVIER, AMSTERDAM, NL, vol. 520, no. 16, 30 March 2012 (2012-03-30), pages 5322-5327, XP028512954, ISSN: 0040-6090, DOI: 10.1016/J.TSF.2012.03.127 [retrieved on 2012-04-06]
- None

## Description

### BACKGROUND

Electrodeposition is recognized as a low-cost method for forming a dense coating or cladding on a variety of conductive materials, including metals, alloys, conductive polymers and the like. Electrodeposition has also been successfully used to deposit nanolaminated coatings or claddings on non-conductive material such as non-conductive polymers by incorporating sufficient materials into the non-conductive polymer to render it sufficiently conductive or by treating the surface to render it conductive, for example by electroless deposition of nickel, copper, silver, cadmium etc. in a variety of engineering applications.

Electrodeposition has also been demonstrated as a viable means for producing laminated and nanolaminated coatings, claddings, materials and objects, in which the individual laminate layers may vary in the composition of the metal, ceramic, organic-metal composition, and/or microstructure features. Laminated coatings or claddings and materials, and in particular nanolaminated metals, are of interest for a variety of purposes, including structural, thermal, and corrosion resistance applications because of their unique toughness, fatigue resistance, thermal stability, wear, abrasion resistance and chemical properties. Characterization of Cr-Ni multilayers electroplated from a chromium (III) - nickel (II) bath using pulse current is disclosed e.g., in Huang et al., Scripta Mat. 2007, 57, 61-64.

### SUMMARY

The present invention is directed to a process for forming a multilayered coating or cladding on a surface of a conductive substrate or mandrel by electrodeposition, the process comprising: (a) providing an electrolyte solution comprising a nickel salt and a chromium salt; (b) providing the conductive substrate or mandrel for electrodeposition; (c) contacting at least a portion of a surface of the conductive substrate or mandrel with the electrolyte solution; (d) depositing a seed layer of nickel and chromium on the conductive substrate or mandrel by passing a seed layer plating current through the conductive substrate or mandrel for a first time period ranging from about 1 minute to about 10 minutes, the seed layer comprising greater than about 90% nickel by weight; (e) depositing a first layer of a second nickel-chromium alloy by passing a first electric current through the conductive substrate or mandrel for a second time period ranging from about 50 milliseconds to about 500 milliseconds, the first layer comprising from about 5% to about 35% chromium by weight; (f) depositing a second layer of nickel and chromium by passing a second electric current through the conductive substrate or mandrel for a third time period ranging from about 50 milliseconds to about 500 milliseconds, the second layer comprising greater than about 90% nickel by weight; (g) repeating steps (e) and (f) four or more times, thereby producing a multilayered coating or cladding comprising the seed layer and alternating first layers and second layers on the surface of the conductive substrate or mandrel; and (h) optionally separating the mandrel from the cladding.

The present disclosure is directed, among other things, to the production of NiCr nanolaminated materials having a high hardness. The materials have a variety of uses including, but not limited to, the preparation of coatings or claddings that protect an underlying substrate, and which may also increase its strength. In one embodiment hard NiCr coatings or claddings and materials are wear/abrasion resistant and find use as wear resistant coatings or claddings in tribological applications. In another embodiment the hard NiCr coatings or claddings prevent damage to the underlying substrates. Where the NiCr materials are applied as a coating or cladding that is more noble then the underlying material upon which it is placed, it may function as a corrosion resistant barrier coating or cladding.

### DESCRIPTION

### 1.1 Overview

The present disclosure is directed to methods of producing laminate materials, and to coatings or claddings comprising layers each comprising nickel or nickel and chromium. The materials, which are prepared by electrodeposition, have a Vickers hardness greater than about 750 without the addition of other elements or heat treatments.

Some embodiments are directed to an electrodeposition process for forming a multilayered nickel and chromium containing coating or cladding on a substrate or mandrel comprising:
(a) providing an electrolyte solution comprising a nickel salt and/or a chromium salt;
(b) providing a conductive substrate or mandrel for electrodeposition;
(c) contacting at least a portion of the surface of the substrate or mandrel with the electrolyte solution;
(d) passing a seed layer plating current through the substrate or mandrel to deposit a nickel and chromium containing seed layer on the substrate or mandrel, where the seed layer comprises greater than about 90*%* nickel by weight;
(e) passing a first electric current through the substrate or mandrel to deposit a nickel-chromium alloy first layer comprising from about 5 to about 35*%* chromium by weight;
(f) passing a second electric current through the substrate to deposit a nickel and chromium containing second layer comprising greater than about 90*%* nickel by weight; and
(g) repeating steps (e) and (f) four or more times, thereby producing a multilayered coating or cladding having a seed layer and alternating first layers and second layers on the surface of the substrate or mandrel.

The method may further comprise the step of separating said substrate or mandrel from the coating or cladding, where the coating or cladding forms an object comprised of the laminate material.

The high hardness coating or cladding produced by the process typically has alternating first and second layers. In some embodiments, the first layers are each from about 125 nm to about 175 nm thick, and comprise from about 5*%* to about 35*%* chromium by weight with the balance typically comprising nickel, and the second layers are each from about 25 nm to about 75 nm thick, and comprise greater than about 90*%* nickel by weight, with the balance typically comprising chromium. In other embodiments, the percentages of chromium and nickel percentages in the first and second layers may vary outside of the above ranges, and the first and second layers may each be thicker or thinner than the above first- and second-layer thicknesses.

### 1.2 Definitions

"Laminate" or "laminated" as used herein refers to materials that comprise a series of layers, including nanolaminated materials.

"Nanolaminate" or "nanolaminated" as used herein refers to materials that comprise a series of layers less than 1 micron.

All compositions given as percentages are given as percent by weight unless stated otherwise.

### 1.3 Nanolaminate NiCr Coatings and Claddings

### 1.3.1 Nanolaminate NiCr Materials and Coatings or Claddings and Methods of Their Preparation

Electrodeposition has been demonstrated as a viable means for producing nanolaminated metal materials and coatings or claddings in which the individual laminate layers may vary in the composition or structure of the metal components. In addition, electrodeposition permits the inclusion of other components, such as ceramic particles and organic-metal components.

Multi-laminate materials having layers with different compositions can be realized by moving a mandrel or substrate from one bath to another and electrodepositing a layer of the final material. Each bath represents a different combination of parameters, which may be held constant or varied in a systematic manner. Accordingly, laminated materials may be prepared by alternately electroplating a substrate or mandrel in two or more electrolyte baths of differing electrolyte composition and/or under differing plating conditions (*e.g.*, current density and mass transfer control). Alternatively, laminated materials may be prepared using a single electrolyte bath by varying the electrodeposition parameters such as the voltage applied, the current density, mixing rate, substrate or mandrel movement (*e.g.*, rotation) rate, and/or temperature. By varying those and/or other parameters, laminated materials having layers with differing metal content can be produced in a single bath.

Embodiments of the present disclosure provide processes for forming a multilayered nickel and chromium containing coating or cladding on a substrate or mandrel by electrodeposition comprising:
(a) providing an electrolyte solution comprising a nickel salt and/or a chromium salt;
(b) providing a conductive substrate or mandrel for electrodeposition;
(c) contacting at least a portion of the surface of the substrate or mandrel with the electrolyte solution;
(d) passing a seed layer plating current through the substrate or mandrel to deposit a nickel and chromium containing seed layer on the substrate or mandrel, where the seed layer comprises greater than about 90*%* nickel by weight;
(e) passing a first electric current through the substrate or mandrel to deposit a nickel-chromium alloy first layer comprising from about 5 to about 35*%* chromium by weight;
(f) passing a second electric current through the substrate to deposit a nickel and chromium containing second layer comprising greater than about 90*%* nickel by weight; and
(g) repeating steps (e) and (f) four or more times, thereby producing a multilayered coating or cladding having a seed layer and alternating first layers and second layers on the surface of the substrate or mandrel.

Embodiments of the processes herein may additionally comprise a step of separating the substrate or mandrel from the coating or cladding.

Embodiments of the method may additionally comprise, prior to passing said first electric current, a step of dynamically manipulating, at the cathode diffusion layer, the concentration and speciation of chromium ions via applying a seed layer plating current through the substrate; and depositing a nickel-chromium alloy first layer having a surface roughness (arithmetical mean roughness or Ra) of less than 0.1 micrometer (*e.g.*, less than 0.09, 0.08, 0.07, or 0.05 microns) and comprising from about 5*%* to about 35*%* chromium by weight (*e.g.*, about 5*%* to about 10*%*, about 10*%* to about 20*%*, about 10*%* to about 25*%*, or about 20*%* to about 35*%*).

Where separate baths are employed to deposit the first and second layers, step (f) includes contacting at least a portion of the substrate or mandrel having the first layer deposited on it with a second of said one or more electrolyte solutions (baths) prior to passing a second electric current through the substrate, to deposit a second layer comprising a nickel-chromium alloy on the surface.

Where the electroplated material is desired as an object that is "electroformed" or as a material separated from the substrate or mandrel, the method may further comprise a step of separating the substrate or mandrel from the electroplated coating or cladding. Where a step of separating the electroplated material from the substrate or mandrel is to be employed, the use of electrodes (mandrel), such as titanium electrodes (mandrel), that do not form tight bonds with the coating or cladding may be employed.

In embodiments where a single bath is used to deposit the first and second layers, providing one or more electrolyte solutions comprises providing a single electrolyte solution comprising a nickel salt and a chromium salt. The step of passing an electric current through the substrate or mandrel comprises alternately pulsing said electric current for predetermined durations between said first electrical current density and said second electrical current density, where the first electrical current density is effective to electrodeposit a first composition comprising an alloy of nickel and chromium, and the second electrical current density is effective to electrodeposit a second composition comprising nickel or a composition (*e.g.*, an alloy) comprising nickel and chromium. The process is repeated to produce a multilayered alloy having alternating first and second layers on at least a portion of the surface of the substrate or mandrel.

Regardless of whether the laminated material is produced by electroplating in more than one bath (*e.g.*, alternately plating in two different baths) or in a single bath, the electrolytes employed may be aqueous or non-aqueous. Where aqueous baths are employed they may benefit from the addition of one or more, two or more, or three or more complexing agents, which can be particularly useful in complexing chromium in the +3 valency. Among the complexing agents that may be employed in aqueous baths are one or more of citric acid, ethylenediaminetetraacetic acid (EDTA), triethanolamine (TEA), ethylenediamine (En), formic acid, acetic acid, hydroxyacetic acid, malonic acid, or an alkali metal salt or ammonium salt of any thereof. In some embodiments, the electrolyte used in plating comprises a Cr⁺³ salt (*e.g.*, a tri-chrome plating bath). In other embodiments, the electrolyte used in plating comprises either Cr⁺³ and one or more complexing agents selected from citric acid, formic acid, acetic acid, hydroxyacetic acid, malonic acid, or an alkali metal salt or ammonium salt of any thereof. In still other embodiments, the electrolyte used in plating comprises either Cr⁺³ and one or more amine containing complexing agents selected from EDTA, TEA, En, or a salt of any thereof.

The temperature at which the electrodeposition process is conducted may alter the composition of the electrodeposit. Where the electrolyte(s) employed are aqueous, the electrodeposition process will typically be kept in the range of about 18° C to about 45° C (*e.g.*, 18° C to about 35° C) for the deposition of both the first and second layers.

Both potentiostatic and galvanostatic control of the electrodeposition of the first and second layers is possible regardless of whether those layers are applied from different electrolyte baths or from a single bath. In some embodiments, a single electrolyte bath is employed and the first electrical current ranges from about 100 to about 300 mA/cm² for the deposition of the first layers, and the second electrical current ranges from about 20 to about 60 mA/cm² for the deposition of the second layers. According to the invention the first electrical current is applied to the substrate or mandrel for about 50 milliseconds to about 500 milliseconds, and the second electrical current is applied to the substrate or mandrel for about 50 milliseconds to about 500 milliseconds. In other embodiments, wherein alternating Ni and/or Ni/Cr containing layers are electrodeposited, the electrodeposition may employ periods of DC plating followed by periods of pulse plating. In embodiments, plating of a nearly pure nickel layer may be conducted either by direct current or by pulse plating.

In such embodiments, the first electrical current is applied to the substrate or mandrel in a pulse ranging from about 50 milliseconds to about 500 milliseconds at a current density of about 100 to about 300 mA/cm2, and the second electrical current is applied to the substrate or mandrel in a pulse ranging from about 50 milliseconds to about 500 milliseconds at a current density from about 20 to about 60 mA/cm². In such embodiments, the resulting coating or cladding has layers of substantially pure nickel alternated with layers of nickel and chromium.

Prior to applying the first and second layers, a seed layer comprising greater than about 90% nickel by weight (*e.g.*, about 90.00 up to about 100, about 90 to about 92, about 92 to about 95, about 94 to about 98, about 95 up to about 100, about 96 to about 100, about 97.00 to about 99.99, about 98.00 to about 99.99, about 99.00 to about 99.99) is applied to the substrate or mandrel for a first time period ranging from about 1 minute to about 10 minutes . Where a strike layer is also applied, the strike layer is applied prior to the seed layer.

To ensure adequate binding of NiCr coatings or claddings to substrates, it is necessary to prepare the substrate for electrodeposition (*e.g.*, the surface must be clean and electrochemically active, and the roughness determined to be in an adequate range). In addition, depending on the substrate it may be desirable to employ a strike layer, particularly where the substrate is a polymer or plastic that has previously been rendered conductive by electroless plating or by chemical conversion of its surface, as in the case for zincate processing of aluminum, which is performed prior to the electroless or electrified deposition. Where a strike layer is applied, it may be chosen from any of a number of metals including, but not limited to, copper, nickel, zinc, cadmium, platinum etc. In some embodiments, the strike layer is nickel or a nickel alloy from about 100 nm to about 1,000 nm or from about 250 nm to about 2,500 nm thick. In other embodiments, where the substrate is a non-conductive polymeric material rendered conductive by electroless deposition of a metal, the metal composition deposited by the electroless plating may act as a strike layer.

The hard nanolaminate materials, such as coatings and claddings, produced by the processes described above will typically comprise alternating first and second layers in addition to a seed layer and any strike layer applied to the substrate. The first layers each have a thickness independently selected from the following ranges: from about 25 nm to about 75 nm, from about 25 nm to about 50 nm, from about 35 nm to about 65 nm, from about 40 nm to about 60 nm, or from about 50 nm to about 75 nm. The second layers each have a thickness independently selected from the following ranges: from about 75 nm to about 225 nm, from about 100 to about 200 nm, from about 125 nm to about 175 nm, from about 125 nm to about 150 nm, from about 135 nm to about 165 nm, from about 140 nm to about 160 nm, or from about 150 nm to about 175 nm.

First layers may typically comprise a percent of chromium by weight selected from one of the following ranges: from about 7 to about 32*%*, from about 10 to about 30*%*, from about 12 to about 28*%*, from about 10 to about 32*%*, from about 10 to about 18*%*, from about 10 to about 16*%*, from about 9 to about 17*%*, from about 9 to about 19*%*, from about 20 to about 32*%*, from about 10 to about 20*%*, from about 15 to about 30*%*, from about 16 to about 25*%*, and from about 18 to about 27*%*. The balance of first layers may be nickel, or may comprise nickel and one or more, two or more, three or more, or four or more additional elements selected independently for each second layer, e.g., from elements such as C, Co, Cu, Fe, In, Mn, Mo, P, Nb, Ni and W. In some embodiments, the balances of the first layers each independently comprise nickel and one or more, two or more, or three or more, elements selected independently for each layer from C, Co, Cr, Cu, Mo, P, Fe, Ti, and W (*e.g.*, C, Co, Cr, Cu, Mo, P, Fe, and W, or alternatively, Co, Cr, Cu, Mo, Fe, and W).

Second layers may typically comprise a percent of nickel by weight in one of the following ranges: about 90.00 up to about 100*%*, about 90 to about 92*%*, about 92 to about 95*%*, about 94 to about 98*%*, about 96 up to about 100*%*, about 97.00 to about 99.99*%*, about 98.00 to about 99.99*%*, and about 99.00 to about 99.99*%*. The balance of second layers may be chromium, or may be comprised of one or more, two or more, three or more, or four or more additional elements selected independently for each second layer, e.g., from elements such as C, Co, Cr, Cu, Fe, In, Mn, Nb, Sn, W, Mo, and P. In some embodiments, the balances of the second layers each independently comprise chromium and one or more additional elements selected independently for each layer, e.g. from elements such as C, Co, Cu, Fe, Ni, W, Mo and/or P. In the embodiments described herein, for any such additional element to be considered as being present, it must be present in the electrodeposited material in a non-trivial amount, *i.e.*, not less than an amount selected from the following amounts: 0.005*%*, 0.01*%*, 0.05*%* or 0.1*%* by weight.

Laminated or nanolaminated materials including coatings and claddings prepared as described herein comprise two or more, three or more, four or more, six or more, eight or more, ten or more, twenty or more, forty or more, fifty or more, 100 or more, 200 or more, 500 or more or 1,000 or more alternating first and second layers. In such embodiments, the first and second layers are counted as pairs of first and second layers. Accordingly, two layers each having a first layer and a second layer, consists of a total of four laminate layers (*i.e.*, each layer is counted separately).

In addition to the methods of preparing hard NiCr materials, the present disclosure is directed to hard NiCr materials, including hard NiCr coatings or claddings and electroformed NiCr objects, prepared by the methods described above.

### 1.3.2 Properties and Applications of Nanolaminate NiCr Coatings or Claddings

### 1.3.2.1 Surface Properties

Embodiments of the hard NiCr materials described herein have a number of properties that render them useful for both industrial and decorative purposes. The coatings or claddings applied are self-leveling and, depending on the exact composition of the outermost layer, can be reflective to visible light. Accordingly, the hard NiCr materials may serve as replacements for chrome finishes in a variety of applications where reflective metal surfaces are desired. Such applications include, but are not limited to, mirrors, automotive details such as bumpers or fenders, decorative finishes and the like.

In some embodiments, the laminated NiCr coatings or claddings described herein have a surface roughness (arithmetical mean roughness or Ra) of less than 0.1 micrometer (*e.g.*, 0.09, 0.08, 0.07, or 0.05 microns).

### 1.3.2.2 Hardness

Through the use of nanolamination, it is possible to increase the hardness of NiCr alloys above the hardness observed for homogeneous electrodeposited NiCr compositions (alloys) that have not been heat treated and have the same thickness and average composition as the hard NiCr nanolaminate material. Embodiments of the laminated NiCr materials disclosed herein have a Vickers hardness (microhardness) number as measured by ASTM E384-11e1 in a range selected from: 550-750, 550-600, 600-650, 650-700, 700-750, 750-1000, 1000-1100, 1100 to 1200, or 1200 or more; or, alternatively, a hardness number greater than 750, 800, 850, 900, 950, 1000, 1050, 1100, 1150, 1200, or more, without heat treatment. The use of heat treatments in the presence of other elements such as B, P, or C in the first and second layers can increase the hardness of the coating or cladding.

In other embodiments, the NiCr materials described herein comprise alternating first and second layers that consist essentially of nickel or a nickel-chromium alloy. Such materials have a Vickers microhardness as measured by ASTM E384-11e1 of 550-750, 550-600, 600-650, 650-700, 700-750, 750-800, 800-850, 850-900, 900-1000, 1000-1100, 1100 to 1200, or 1200 or more without heat treatment.

In some embodiments, the NiCr materials described herein consist of alternating first and second layers that consist of nickel or a nickel-chromium alloy. Such materials have a Vickers microhardness as measured by ASTM E384-11e1 in a range selected from 550-750, 550-600, 600-650, 650-700, 700-750, 750-800, 800-850, 850-900, 900-1,000 or 1,000-1,100 without heat treatment.

### 1.3.2.3 Abrasion Resistance

Due to their high hardness, embodiments of the laminated NiCr materials disclosed herein are useful as a means of providing resistance to abrasion, especially when they are employed as coatings or claddings. When subjected to testing on a Taber Abraser equipped with CS-10 wheels and a 250 g load and operated at room temperature at the same speed for both samples (*e.g.*, 95 RPM), embodiments of the nanolaminate NiCr coatings or claddings disclosed herein that have not been heat treated display 5*%*, 10*%*, 20*%*, 30*%* or 40*%* less loss of weight than homogeneous electrodeposited NiCr compositions (alloys) that have not been heat treated and have the same thickness and average composition as the hard NiCr nanolaminate material. In other embodiments, the laminated NiCr compositions display a higher abrasion resistance when subject to testing under ASTM D4060 than their homogeneous counterpart (*e.g.*, homogeneous electrodeposited counterpart having the average composition of the laminated NiCr composition).

### 1.3.2.4 Corrosion protection

The behavior of organic, ceramic, metal and metal-containing coatings or claddings in corrosive environments depends primarily on their chemistry, microstructure, adhesion, thickness and galvanic interaction with the substrate to which they are applied.

NiCr generally acts as a barrier coating or cladding, being more electronegative (more noble) than substrates to which it will be applied, such as iron-based substrates. As such, NiCr coatings or claddings act by forming a barrier to oxygen and other agents (*e.g.*, water, acid, base, salts, and/or H₂S) that can cause corrosive damage, including oxidative corrosion. When a barrier coating or cladding that is more noble than its underlying substrate is marred or scratched, or if coverage is not complete, the coatings or claddings will not work and may accelerate the progress of substrate corrosion at the substrate-coating or cladding interface, resulting in preferential attack of the substrate. Consequently, embodiments of the coatings or claddings prepared from the hard NiCr coatings or claddings described herein offer advantages over softer NiCr nanolaminate coatings or claddings as they are less likely to permit a scratch to reach the surface of a corrosion susceptible substrate. Another advantage offered by some embodiments of the hard NiCr laminate coatings or claddings described herein are their fully dense structure, which lacks any significant pores or micro-cracks that extend from the surface of the coating or cladding to the substrate. In some embodiments, to avoid the formation of microcracks, the first layer can be a nickel rich ductile layer that hinders the formation of continuous cracks from the coating or cladding surface to the substrate. To the extent that microcracks occur in the high chromium layers, they can be small and tightly spaced. The lack of pores and continuous microcracks more effectively prohibits corrosive agents from reaching the underlying substrate and renders the laminate NiCr coatings or claddings described herein more effective as barrier coatings or claddings to oxidative damage of a substrate than an equivalent thickness of electrodeposited chromium.

### 2.0 Certain Embodiments

Disclosed is a process for forming a multilayered coating or cladding on a surface of a conductive substrate or mandrel by electrodeposition, the process comprising: (a) providing an electrolyte solution comprising a nickel salt and a chromium salt; (b) providing the conductive substrate or mandrel for electrodeposition; (c) contacting at least a portion of a surface of the conductive substrate or mandrel with the electrolyte solution; (d) depositing a seed layer of nickel and chromium on the conductive substrate or mandrel by passing a seed layer plating current through the conductive substrate or mandrel for a first time period ranging from about 1 minute to about 10 minutes, the seed layer comprising greater than about 90*%* nickel by weight; (e) depositing a first layer of a second nickel-chromium alloy by passing a first electric current through the conductive substrate or mandrel for a second time period ranging from about 50 milliseconds to about 500 milliseconds, the first layer comprising from about 5*%* to about 35*%* chromium by weight; (f) depositing a second layer of nickel and chromium by passing a second electric current through the conductive substrate or mandrel for a third time period ranging from about 50 milliseconds to about 500 milliseconds, the second layer comprising greater than about 90*%* nickel by weight; (g) repeating steps (e) and (f) four or more times, thereby producing a multilayered coating or cladding comprising the seed layer and alternating first layers and second layers on the surface of the conductive substrate or mandrel; and (h) optionally separating the mandrel from the cladding,
optionally wherein the seed layer plating current has a density selected from the group consisting of from about 20 to about 60 mA/cm², from about 20 to about 50 mA/cm², from about 30 to about 60 mA/cm², from about 30 to about 50 mA/cm², from about 25 to about 55 mA/cm², from about 20 to about 45 mA/cm², from about 20 to about 35 mA/cm², from about 30 to about 45 mA/cm², from about 30 to about 40 mA/cm², and from about 40 to about 50 mA/cm² and/or
optionally wherein the seed layer plating current has a density selected from the group consisting of about 20 mA/cm², about 25 mA/cm², about 30 mA/cm², about 35 mA/cm², about 40 mA/cm², about 45 mA/cm², about 50 mA/cm², about 55 mA/cm², and about 60 mA/cm² and/or
optionally wherein the seed layer plating current is applied to the substrate or mandrel for a time period selected from the group consisting of about 1 minute to about 5 minutes, about 3 minutes to about 8 minutes, about 5 minutes to about 10 minutes, about 2 minutes to about 6 minutes, about 4 minutes to about 8 minutes, and about 6 minutes to about 10 minutes and/or
optionally wherein the seed layer comprises nickel in a weight percent (Ni wt.*%*) range selected from the group consisting of about 90 to about 92, about 92 to about 95, about 94 to about 98, about 95 up to about 100, about 96 to about 100, about 97.00 to about 99.99, about 98.00 to about 99.99, and about 99.00 to about 99.99 and/or
optionally wherein the first electric current has a density in a range selected from the group consisting of from about 100 to about 300 mA/cm², from about 100 to about 200 mA/cm², from about 200 to about 300 mA/cm², from about 150 to about 250 mA/cm², from about 150 to about 290 mA/cm², and from about 160 to about 280 mA/cm² and/or
optionally wherein the first electric current has a density selected from the group consisting of about 160 mA/cm², about 180 mA/cm², about 200 mA/cm², about 220 mA/cm², about 240 mA/cm², and about 260 mA/cm² and/or
optionally wherein the first current is applied for a time period selected from the group consisting of about 50 milliseconds to about 100 milliseconds, about 100 milliseconds to about 200 milliseconds, about 200 milliseconds to about 300 milliseconds, about 200 milliseconds to about 400 milliseconds, about 300 milliseconds to about 400 milliseconds, about 400 milliseconds to about 500 milliseconds, and about 100 milliseconds to about 400 milliseconds and/or
optionally wherein the second electric current has a density in a range selected from the group consisting of from about 20 to about 60 mA/cm², from about 20 to about 50 mA/cm², from about 30 to about 60 mA/cm², from about 30 to about 50 mA/cm², from about 25 to about 55 mA/cm², from about 20 to about 45 mA/cm², from about 20 to about 35 mA/cm², from about 30 to about 45 mA/cm², from about 30 to about 40 mA/cm², and from about 40 to about 50 mA/cm² and/or
optionally wherein the second electric current has a density selected from the group consisting of about 20 mA/cm², about 25 mA/cm², about 30 mA/cm², about 35 mA/cm², about 40 mA/cm², about 45 mA/cm². about 50 mA/cm². about 55 mA/cm², and about 60 mA/cm² and/or
optionally wherein the second electric current is applied for a time period selected from the group consisting of: about 50 milliseconds to about 500 milliseconds, about 50 milliseconds to about 100 milliseconds, about 100 milliseconds to about 200 milliseconds, about 200 milliseconds to about 300 milliseconds, about 200 milliseconds to about 400 milliseconds, about 300 milliseconds to about 400 milliseconds, about 400 milliseconds to about 500 milliseconds, and about 100 milliseconds to about 400 milliseconds and/or
optionally where steps (e) and (f) are repeated greater than 10, 20, 50, 100, 200, 400, 500, 1,000, 2,000, 5,000, 7,500, or 10,000 times and/or
optionally where steps (e) and (f) are repeated from about 4 to 10,000 times, from about 5 to 5,000 times, from about 5 to 2,500 times, and from about 5 to 2,000 times and/or
optionally wherein one, two, three, four or more of the first layers comprises chromium in a weight percent (Cr wt.*%*) range selected from the group consisting of from about 7 to about 32, from about 10 to about 30, from about 12 to about 28, from about 10 to about 32, from about 10 to about 18, from about 10 to about 16, from about 9 to about 17, from about 9 to about 19, from about 20 to about 32, from about 10 to about 20, from about 15 to about 30, from about 16 to about 25, and from about 18 to about 27 and/or
optionally wherein each of the first layers comprises chromium in a weight percent (Cr wt.*%*) range selected from the group consisting of from about 5 to about 35, from about 10 to about 30, from about 12 to about 28, from about 10 to about 32, from about 10 to about 18, from about 10 to about 16, from about 9 to about 17, from about 9 to about 19, from about 20 to about 32, from about 10 to about 20, from about 15 to about 30, from about 16 to about 25, and from about 18 to about 27 and/or
optionally wherein one, two, three, four or more of the second layers comprises nickel in a weight percent (Ni wt.*%*) range selected from the group consisting of about 90.00 up to about 100, about 90 to about 92, about 92 to about 95, about 94 to about 98, about 95 up to about 100, about 96 up to about 100, about 97.00 to about 99.99, about 98.00 to about 99.99, and about 99.00 to about 99.99 and/or
optionally wherein each of the second layers comprises nickel in a weight percent (Ni wt.*%*) range selected from the group consisting of about 90.00 up to about 100, about 90 to about 92, about 92 to about 95, about 94 to about 98, about 96 up to about 100, about 97.00 to about 99.99, about 98.00 to about 99.99, and about 99.00 to about 99.99.

Also described is a process for forming a multilayered coating or cladding on a surface of a substrate or mandrel by electrodeposition, comprising:
(a) providing an electrolyte solution comprising a nickel salt and/or a chromium salt from which nickel and/or chromium can be electrodeposited;
(b) providing a conductive substrate or mandrel for electrodeposition;
(c) contacting at least a portion of the surface of the substrate or mandrel with the electrolyte solution;
(d) passing a seed layer plating current having a density of about 30 to about 50 mA/cm² for a time period of about 1 minute to about 5 minutes through the substrate or mandrel to deposit a nickel and chromium containing seed layer on the substrate or mandrel, where the seed layer comprises greater than about 90*%* nickel by weight;
(e) passing a first electric current having a density of about 100 to about 300 mA/cm² for a time period of about 200 milliseconds to about 400 milliseconds through the substrate or mandrel to deposit a nickel-chromium alloy first layer comprising from about 5 to about 35*%* chromium by weight;
(f) passing a second electric current having a density of about 30 to about 50 mA/cm² for a time period of about 200 milliseconds to about 400 milliseconds through the substrate to deposit a nickel and chromium containing second layer comprising greater than about 90*%* nickel by weight;
(g) repeating steps (e) and (f) 10 or more times, thereby producing a multilayered coating or cladding having a seed layer and alternating first layers and second layers on the surface of the substrate or mandrel; and
(h) optionally separating the substrate or mandrel from the coating or cladding ,
or a process for forming a multilayered coating or cladding on a surface of a substrate or mandrel by electrodeposition, comprising:
(a) providing an electrolyte solution comprising a nickel salt and/or a chromium salt from which nickel and/or chromium can be electrodeposited;
(b) providing a conductive substrate or mandrel for electrodeposition;
(c) contacting at least a portion of the surface of the substrate or mandrel with the electrolyte solution;
(d) passing a seed layer plating current having a density of about 35 to about 45 mA/cm² for a time period of about 1 minute to about 3 minutes through the substrate or mandrel to deposit a nickel and chromium containing seed layer on the substrate or mandrel, where the seed layer comprises greater than about 90*%* nickel by weight;
(e) passing a first electric current having a density of about 150 to about 260 mA/cm² for a time period of about 250 milliseconds to about 350 milliseconds through the substrate or mandrel to deposit a nickel-chromium alloy first layer comprising from about 5 to about 35*%* chromium by weight;
(f) passing a second electric current having a density of about 35 to about 45 mA/cm² for a time period of about 250 milliseconds to about 350 milliseconds through the substrate to deposit a nickel and chromium containing second layer comprising greater than about 90*%* nickel by weight;
(g) repeating steps (e) and (f) 10 or more times, thereby producing a multilayered coating or cladding having a seed layer and alternating first layers and second layers on the surface of the substrate or mandrel; and
(h) optionally separating the substrate or mandrel from the coating or cladding and/or
   optionally wherein one, two, three, four or more of the first layers comprises chromium in a weight percent (Cr wt.*%*) range of from about 12 to 26 and/or
   optionally wherein one, two, three, four or more of the second layers comprises nickel in a weight percent (Ni wt.*%*) range of at least 95*%*.

## Claims

1. A process for forming a multilayered coating or cladding on a surface of a conductive substrate or mandrel by electrodeposition, the process comprising:
(a) providing an electrolyte solution comprising a nickel salt and a chromium salt;
(b) providing the conductive substrate or mandrel for electrodeposition;
(c) contacting at least a portion of a surface of the conductive substrate or mandrel with the electrolyte solution;
(d) depositing a seed layer of nickel and chromium on the conductive substrate or mandrel by passing a seed layer plating current through the conductive substrate or mandrel for a first time period ranging from about 1 minute to about 10 minutes, the seed layer comprising greater than about 90% nickel by weight;
(e) depositing a first layer of a second nickel-chromium alloy by passing a first electric current through the conductive substrate or mandrel for a second time period ranging from about 50 milliseconds to about 500 milliseconds, the first layer comprising from about 5% to about 35% chromium by weight;
(f) depositing a second layer of nickel and chromium by passing a second electric current through the conductive substrate or mandrel for a third time period ranging from about 50 milliseconds to about 500 milliseconds, the second layer comprising greater than about 90% nickel by weight;
(g) repeating steps (e) and (f) four or more times, thereby producing a multilayered coating or cladding comprising the seed layer and alternating first layers and second layers on the surface of the conductive substrate or mandrel; and
(h) optionally separating the mandrel from the cladding.

2. The process of claim 1, wherein the seed layer plating current has a density ranging from about 20 to about 60 mA/cm².

3. The process of claim 1, wherein the seed layer plating current has a density selected from the group consisting of about 20 mA/cm², about 25 mA/cm², about 30 mA/cm², about 35 mA/cm², about 40 mA/cm², about 45 mA/cm², about 50 mA/cm², about 55 mA/cm², and about 60 mA/cm²; and/or
wherein the first electric current has a density selected from the group consisting of about 160 mA/cm², about 180 mA/cm², about 200 mA/cm², about 220 mA/cm², about 240 mA/cm², and about 260 mA/cm²; or
wherein the second electric current has a density selected from the group consisting of about 20 mA/cm², about 25 mA/cm², about 30 mA/cm², about 35 mA/cm², about 40 mA/cm², about 45 mA/cm², about 50 mA/cm², about 55 mA/cm², and about 60 mA/cm².

4. The process of any of claims 1-3 wherein the seed layer comprises from about 90.00% to about 99.99% nickel by weight.

5. The process of any of claims 1, 2 or 4, wherein the first electric current has a density ranging from about 100 mA/cm² to about 300 mA/cm².

6. The process of any of claims 1-4, wherein the second electric current has a density in a range from about 20 mA/cm² to about 60 mA/cm².

7. The process of any of claims 1-4, where steps (e) and (f) are repeated greater than 50 times.

8. The process of any of claims 1-4, where steps (e) and (f) are repeated from about 4 times to 10 000 times.

9. The process of any of claims 1-4, wherein two or more of the first layers comprise from about 7% to about 32% chromium by weight; or
wherein two or more of the second layers comprise from about 90.00% to about 99.99% nickel by weight.

10. The process of any of claims 1-4, wherein each of the first layers comprises from about 5% to about 35% chromium by weight; or
wherein each of the second layers comprises from about 90.00% to about 99.99% nickel by weight.

11. The process of any of claims 1-4, wherein the conductive substrate comprises a non-conductive polymeric material and a conductive metal strike layer.

12. The process of claim 1, wherein the electrolyte solution comprises the nickel salt and/or the chromium salt from which nickel and/or chromium can be electrodeposited;
wherein the depositing the seed layer of nickel and chromium on the conductive substrate or mandrel comprises passing the seed layer plating current having a density of about 30 mA/cm² to about 50 mA/cm² through the conductive substrate or mandrel for a time period of about 1 minute to about 5 minutes;
wherein the depositing the first layer of the nickel-chromium alloy comprises passing the first electric current having a density of about 100 mA/cm² to about 300 mA/cm² through the conductive substrate or mandrel for a time period of about 200 milliseconds to about 400 milliseconds;
wherein the depositing the second layer of nickel and chromium comprises passing the second electric current having a density of about 30 mA/cm² to about 50 mA/cm² through the conductive substrate or mandrel for a time period of about 200 milliseconds to about 400 milliseconds; and
wherein steps (e) and (f) are repeated 10 or more times.

13. The process of claim 1, wherein the electrolyte solution comprises the nickel salt and/or the chromium salt from which nickel and/or chromium can be electrodeposited;
wherein the depositing the seed layer of nickel and chromium on the conductive substrate or mandrel comprises passing the seed layer plating current having a density of about 35 mA/cm² to about 45 mA/cm² through the conductive substrate or mandrel for a time period of about 1 minute to about 3 minutes;
wherein the depositing the first layer of the nickel-chromium alloy comprises passing the first electric current having a density of about 150 mA/cm² to about 260 mA/cm² through the conductive substrate or mandrel for a time period of about 250 milliseconds to about 350 milliseconds;
wherein the depositing the second layer of nickel and chromium comprises passing the second electric current having a density of about 35 mA/cm² to about 45 mA/cm² through the conductive substrate or mandrel for a time period of about 250 milliseconds to about 350 milliseconds; and
wherein steps (e) and (f) are repeated 10 or more times.

14. The process according to claim 12 or 13, wherein two or more of the first layers comprise from about 12% to 26% chromium by weight; or
wherein two or more of the second layers comprise at least 95% nickel by weight.

## Patentansprüche

1. Verfahren zum Bilden einer mehrschichtigen Beschichtung oder Umhüllung auf einer Oberfläche eines leitenden Substrats oder Dorns durch Elektroabscheidung, wobei das Verfahren umfasst:
(a) Bereitstellen einer Elektrolytlösung, die ein Nickelsalz und ein Chromsalz umfasst;
(b) Bereitstellen des leitfähigen Substrats oder Dorns für die Elektroabscheidung;
(c) Inkontaktbringen mindestens eines Teils einer Oberfläche des leitfähigen Substrats oder Dorns mit der Elektrolytlösung;
(d) Abscheiden einer Keimschicht aus Nickel und Chrom auf dem leitfähigen Substrat oder Dorn durch Durchleiten eines Keimschicht-Plattierungsstroms durch das leitfähige Substrat oder den Dorn für eine erste Zeitspanne im Bereich von etwa 1 Minute bis etwa 10 Minuten, wobei die Keimschicht mehr als etwa 90 Gew.-% Nickel umfasst;
(e) Abscheiden einer ersten Schicht aus einer zweiten Nickel-Chrom-Legierung durch Durchleiten eines ersten elektrischen Stroms durch das leitfähige Substrat oder den Dorn für eine zweite Zeitspanne im Bereich von etwa 50 Millisekunden bis etwa 500 Millisekunden, wobei die erste Schicht etwa 5 bis etwa 35 Gew.-% Chrom umfasst;
(f) Abscheiden einer zweiten Schicht aus Nickel und Chrom durch Durchleiten eines zweiten elektrischen Stroms durch das leitfähige Substrat oder den Dorn während einer dritten Zeitspanne im Bereich von etwa 50 Millisekunden bis etwa 500 Millisekunden, wobei die zweite Schicht mehr als etwa 90 Gew.-% Nickel umfasst;
(g) vier- oder mehrmaliges Wiederholen der Schritte (e) und (f), wodurch eine mehrschichtige Beschichtung oder Umhüllung erzeugt wird, die die Keimschicht und abwechselnden ersten Schichten und zweiten Schichten auf der Oberfläche des leitfähigen Substrats oder Dorns umfasst; und
(h) optionales Trennen des Dorns von der Umhüllung.

2. Verfahren nach Anspruch 1, wobei der Keimschicht-Plattierungsstrom eine Dichte im Bereich von etwa 20 bis etwa 60 mA/cm2 aufweist.

3. Verfahren nach Anspruch 1, wobei der Keimschicht-Plattierungsstrom eine Dichte aufweist, die aus der Gruppe ausgewählt ist, die aus etwa 20 mA/cm², etwa 25 mA/cm², etwa 30 mA/cm², etwa 35 mA/cm², etwa 40 mA/cm², etwa 45 mA/cm², etwa 50 mA/cm², etwa 55 mA/cm² und etwa 60 mA/cm² besteht; und/oder
wobei der erste elektrische Strom eine Dichte aufweist, die ausgewählt ist aus der Gruppe bestehend aus etwa 160 mA/cm², etwa 180 mA/cm², etwa 200 mA/cm², etwa 220 mA/cm², etwa 240 mA/cm² und etwa 260 mA/cm²; oder
wobei der zweite elektrische Strom eine Dichte aufweist, die aus der Gruppe ausgewählt ist, bestehend aus etwa 20 mA/cm², etwa 25 mA/cm², etwa 30 mA/cm², etwa 35 mA/cm², etwa 40 mA/cm², etwa 45 mA/cm², etwa 50 mA/cm², etwa 55 mA/cm² und etwa 60 mA/cm².

4. Verfahren nach einem beliebigen der Ansprüche 1-3, wobei die Keimschicht etwa 90,00 bis etwa 99,99 Gew.-% Nickel umfasst.

5. Verfahren nach einem beliebigen der Ansprüche 1, 2 oder 4, wobei der erste elektrische Strom eine Dichte im Bereich von etwa 100 mA/cm² bis etwa 300 mA/cm² aufweist.

6. Verfahren nach einem beliebigen der Ansprüche 1-4, wobei der zweite elektrische Strom eine Dichte im Bereich von etwa 20 mA/cm² bis etwa 60 mA/cm² aufweist.

7. Verfahren nach einem beliebigen der Ansprüche 1-4, wobei die Schritte (e) und (f) mehr als 50 Mal wiederholt werden.

8. Verfahren nach einem beliebigen der Ansprüche 1-4, wobei die Schritte (e) und (f) etwa 4 mal bis 10.000 mal wiederholt werden.

9. Verfahren nach einem beliebigen der Ansprüche 1-4, wobei zwei oder mehr der ersten Schichten etwa 7 bis etwa 32 Gew.-% Chrom umfassen; oder wobei zwei oder mehr der zweiten Schichten etwa 90,00 bis etwa 99,99 Gew.-% Nickel umfassen.

10. Verfahren nach einem beliebigen der Ansprüche 1-4, wobei jede der ersten Schichten etwa 5 bis etwa 35 Gew.-% Chrom umfasst; oder
wobei jede der zweiten Schichten etwa 90,00 Gew.-% bis etwa 99,99 Gew.% Nickel umfasst.

11. Verfahren nach einem beliebigen der Ansprüche 1-4, wobei das leitfähige Substrat ein nicht-leitfähiges Polymermaterial und eine leitfähige Metallschlagschicht umfasst.

12. Verfahren nach Anspruch 1, wobei die Elektrolytlösung das Nickelsalz und/oder das Chromsalz umfasst, aus dem Nickel und/oder Chrom galvanisch abgeschieden werden können;
wobei das Abscheiden der Keimschicht aus Nickel und Chrom auf dem leitfähigen Substrat oder Dorn das Durchleiten des Keimschicht-Plattierungsstroms, der eine Dichte von etwa 30 mA/cm² bis etwa 50 mA/cm² aufweist, durch das leitfähige Substrat oder den Dorn für eine Zeitdauer von etwa 1 Minute bis etwa 5 Minuten umfasst;
wobei das Abscheiden der ersten Schicht der Nickel-Chrom-Legierung das Durchleiten des ersten elektrischen Stroms, der eine Dichte von etwa 100 mA/cm² bis etwa 300 mA/cm² aufweist, durch das leitende Substrat oder den Dorn für eine Zeitdauer von etwa 200 Millisekunden bis etwa 400 Millisekunden umfasst;
wobei das Abscheiden der zweiten Schicht aus Nickel und Chrom das Durchleiten des zweiten elektrischen Stroms, der eine Dichte von etwa 30 mA/cm² bis etwa 50 mA/cm² aufweist, durch das leitende Substrat oder den Dorn für eine Zeitdauer von etwa 200 Millisekunden bis etwa 400 Millisekunden umfasst; und
wobei die Schritte (e) und (f) 10 oder mehr Mal wiederholt werden.

13. Verfahren nach Anspruch 1, wobei die Elektrolytlösung das Nickelsalz und/oder das Chromsalz umfasst, aus dem Nickel und/oder Chrom galvanisch abgeschieden werden kann;
wobei das Abscheiden der Keimschicht aus Nickel und Chrom auf dem leitfähigen Substrat oder Dorn das Durchleiten des Keimschicht-Plattierungsstroms, der eine Dichte von etwa 35 mA/cm² bis etwa 45 mA/cm² aufweist, durch das leitfähige Substrat oder den Dorn für eine Zeitdauer von etwa 1 Minute bis etwa 3 Minuten umfasst;
wobei das Abscheiden der ersten Schicht der Nickel-Chrom-Legierung das Durchleiten des ersten elektrischen Stroms, der eine Dichte von etwa 150 mA/cm² bis etwa 260 mA/cm² aufweist, durch das leitende Substrat oder den Dorn für eine Zeitdauer von etwa 250 Millisekunden bis etwa 350 Millisekunden umfasst;
wobei das Abscheiden der zweiten Schicht aus Nickel und Chrom das Durchleiten des zweiten elektrischen Stroms, der eine Dichte von etwa 35 mA/cm² bis etwa 45 mA/cm² aufweist, durch das leitende Substrat oder den Dorn für eine Zeitdauer von etwa 250 Millisekunden bis etwa 350 Millisekunden umfasst; und
wobei die Schritte (e) und (f) 10 oder mehr Mal wiederholt werden.

14. Verfahren nach Anspruch 12 oder 13, wobei zwei oder mehr der ersten Schichten etwa 12 bis 26 Gew.-% Chrom umfassen; oder
wobei zwei oder mehr der zweiten Schichten mindestens 95 Gew.-% Nickel umfassen.

## Revendications

1. Procédé de formation d'un revêtement ou d'un placage multicouche sur une surface d'un substrat ou mandrin conducteur par électrodéposition, le procédé comprenant :
(a) la fourniture d'une solution d'électrolyte comprenant un sel de nickel et un sel de chrome ;
(b) la fourniture du substrat ou mandrin conducteur pour électrodéposition ;
(c) la mise en contact d'au moins une partie d'une surface du substrat ou mandrin conducteur avec la solution d'électrolyte ;
(d) le dépôt d'une couche d'amorce de nickel et de chrome sur le substrat ou mandrin conducteur par passage d'un courant de placage de couche d'amorce à travers le substrat ou mandrin conducteur pendant une durée d'environ 1 minute à environ 10 minutes, la couche d'amorce comprenant plus d'environ 90 % de nickel en poids ;
(e) le dépôt d'une première couche d'un deuxième alliage nickel-chrome par passage d'un premier courant électrique à travers le substrat ou mandrin conducteur pendant une deuxième durée dans la plage d'environ 50 millisecondes à environ 500 millisecondes, la première couche comprenant d'environ 5 % à environ 35 % de chrome en poids ;
(f) le dépôt d'une deuxième couche de nickel et de chrome par passage d'un deuxième courant électrique à travers le substrat ou mandrin conducteur pendant une troisième durée dans la plage d'environ 50 millisecondes à environ 500 millisecondes, la deuxième couche comprenant plus d'environ 90 % de nickel en poids ;
(g) la répétition des étapes (e) et (f) quatre fois ou plus, de façon à produire un revêtement ou placage multicouche comprenant la couche d'amorce et des premières couches et des deuxième couches alternées sur la surface du substrat ou mandrin conducteur ; et
(h) facultativement, la séparation du mandrin du placage.

2. Procédé selon la revendication 1, dans lequel le courant de placage de couche d'amorce a une densité dans la plage d'environ 20 à environ 60 mA/cm².

3. Procédé selon la revendication 1, dans lequel le courant de placage de couche d'amorce a une densité choisie dans le groupe constitué d'environ 20 mA/cm², environ 25 mA/cm², environ 30 mA/cm², environ 35 mA/cm², environ 40 mA/cm², environ 45 mA/cm², environ 50 mA/cm², environ 55 mA/cm², et environ 60 mA/cm² ; et/ou dans lequel le premier courant électrique a une densité choisie dans le groupe constitué d'environ 160 mA/cm², environ 180 mA/cm², environ 200 mA/cm², environ 220 mA/cm², environ 240 mA/cm², et environ 260 mA/cm² ; ou dans lequel le deuxième courant électrique a une densité choisie dans le groupe constitué d'environ 20 mA/cm², environ 25 mA/cm², environ 30 mA/cm², environ 35 mA/cm², environ 40 mA/cm², environ 45 mA/cm², environ 50 mA/cm², environ 55 mA/cm² et environ 60 mA/cm².

4. Procédé selon l'une quelconque des revendications 1 à 3 dans lequel la couche d'amorce comprend d'environ 90,00 % à environ 99,99 % de nickel en poids.

5. Procédé selon l'une quelconque des revendications 1,2 ou 4, dans lequel le premier courant électrique a une densité dans la plage d'environ 100 mA/cm² à environ 300 mA/cm².

6. Procédé selon l'une quelconque des revendications 1 à 4, dans lequel le deuxième courant électrique a une densité dans une plage d'environ 20 mA/cm² à environ 60 mA/cm².

7. Procédé selon l'une quelconque des revendications 1 à 4, où les étapes (e) et (f) sont répétées plus de 50 fois.

8. Procédé selon l'une quelconque des revendications 1 à 4, où les étapes (e) et (f) sont répétées d'environ 4 fois à 10 000 fois.

9. Procédé selon l'une quelconque des revendications 1 à 4, dans lequel deux ou plus des premières couches comprennent d'environ 7 % à environ 32 % de chrome en poids ; ou dans lequel deux ou plus des deuxièmes couches comprennent d'environ 90,00 % à environ 99,99 % de nickel en poids.

10. Procédé selon l'une quelconque des revendications 1 à 4, dans lequel chacune des premières couches comprend d'environ 5 % à environ 35 % de chrome en poids ; ou
dans lequel chacune des deuxièmes couches comprennent d'environ 90,00 % à environ 99,99 % de nickel en poids.

11. Procédé selon l'une quelconque des revendications 1 à 4, dans lequel le substrat conducteur comprend un matériau polymère non conducteur et une couche d'amorce de métal conducteur.

12. Procédé selon la revendication 1, dans lequel la solution d'électrolyte comprend le sel de nickel et/ou le sel de chrome à partir duquel du nickel et/ou du chrome peut être électrodéposé ;
dans lequel le dépôt de la couche d'amorce de nickel et de chrome sur le substrat ou mandrin conducteur comprend le passage du courant de placage de couche d'amorce ayant une densité d'environ 30 mA/cm² à environ 50 mA/cm² à travers le substrat ou mandrin conducteur pendant une durée d'environ 1 minute à environ 5 minutes ;
dans lequel le dépôt de la première couche de l'alliage nickel-chrome comprend le passage du premier courant électrique ayant une densité d'environ 100 mA/cm² à environ 300 mA/cm² à travers le substrat ou mandrin conducteur pendant une durée d'environ 200 millisecondes à environ 400 millisecondes ;
dans lequel le dépôt de la deuxième couche de nickel et de chrome comprend le passage du deuxième courant électrique ayant une densité d'environ 30 mA/cm² à environ 50 mA/cm² à travers le substrat ou mandrin conducteur pendant une durée d'environ 200 millisecondes à environ 400 millisecondes ; et dans lequel les étapes (e) et (f) sont répétées 10 fois ou plus.

13. Procédé selon la revendication 1, dans lequel la solution d'électrolyte comprend le sel de nickel et/ou le sel de chrome à partir duquel du nickel et/ou du chrome peut être électrodéposé ;
dans lequel le dépôt de la couche d'amorce de nickel et de chrome sur le substrat ou mandrin conducteur comprend le passage du courant de placage de couche d'amorce ayant une densité d'environ 35 mA/cm² à environ 45 mA/cm² à travers le substrat ou mandrin conducteur pendant une durée d'environ 1 minute à environ 3 minutes ;
dans lequel le dépôt de la première couche de l'alliage nickel-chrome comprend le passage du premier courant électrique ayant une densité d'environ 150 mA/cm² à environ 260 mA/cm² à travers le substrat ou mandrin conducteur pendant une durée d'environ 250 millisecondes à environ 350 millisecondes ;
dans lequel le dépôt de la deuxième couche de nickel et de chrome comprend le passage du deuxième courant électrique ayant une densité d'environ 35 mA/cm² à environ 45 mA/cm² à travers le substrat ou mandrin conducteur pendant une durée d'environ 250 millisecondes à environ 350 millisecondes ; et dans lequel les étapes (e) et (f) sont répétées 10 fois ou plus.

14. Procédé selon la revendication 12 ou 13, dans lequel deux ou plus des premières couches comprennent d'environ 12 % à 26 % de chrome en poids ; ou dans lequel deux ou plus des deuxièmes couches comprennent au moins 95 % de nickel en poids.
